

[54] **MIXING PROCESS AND EXTRUSION  
OF SOLID PROPELLANTS**

[75] Inventor: **Martin H. Kaufman**, China Lake, Calif.

[73] Assignee: **The United States of America as  
represented by the Secretary of the  
Navy**

[22] Filed: **June 11, 1968**

[21] Appl. No.: **738,721**

**Related U.S. Application Data**

[63] Continuation of Ser. No. 361,612, April 17, 1964.

[52] **U.S. Cl.** ..... **264/3 B, 149/22, 149/40,  
149/41, 149/42, 149/43, 149/44**

[51] **Int. Cl.** ..... **C06b 21/02**

[58] **Field of Search** ..... **264/3; 149/22, 60, 40, 42,  
149/43, 44, 41, 76, 85, 19, 20**

[56]

**References Cited**

**UNITED STATES PATENTS**

|           |         |                     |          |
|-----------|---------|---------------------|----------|
| 3,155,749 | 11/1964 | Rossen et al. ....  | 264/3    |
| 3,351,505 | 11/1967 | Shapiro et al. .... | 149/44   |
| 3,431,154 | 3/1969  | Kelly et al. ....   | 149/44 X |

*Primary Examiner*—Stephen J. Lechert, Jr.  
*Attorney*—George J. Rubens and Roy Miller

[57]

**ABSTRACT**

An improved extrudable, high energy solid propellant composition consisting essentially of the copolymer of vinylidene fluoride and perfluoropropylene (Viton), an inorganic oxidizer such as ammonium perchlorate, potassium perchlorate or ammonium nitrate, and a metal powder such as aluminum, beryllium, magnesium or zirconium. This composition is extrudable into any suitable shape and has a very high percentage theoretical maximum density so as to be practical for utilization in rocket motors for propulsion.

**4 Claims, No Drawings**

## MIXING PROCESS AND EXTRUSION OF SOLID PROPELLANTS

### REFERENCE TO RELATED APPLICATION

This invention is a continuation of U.S. Pat. application Ser. No. 361,612, filed in the U. S. Patent Office on 17 April 1964.

### BACKGROUND OF THE INVENTION

The present invention relates to an improved extrudable, high energy, high density solid propellant and to the method of preparation thereof.

Those concerned with the development of solid propellants have long known and recognized the need for a propellant with a high delivered density-impulse, high temperature stability and good safety characteristics. A propellant of this kind finds greatest use in the system where the propellant burnout mass is very large compared to the propellant volume. As variations in the properties are required for a specific application, variations in the formulation are needed. Propellants presently available have density specific impulse values on the order of 430 - 470 g-sec/cc. The achievement of high density in a composite propellant is controlled by the density and generally the particle size of the ingredients and ultimately the method of fabrication which is limited often by safety features of the processing system. Harsh working of the material may cause ignition.

The present invention attains a very high theoretical density impulse of a value between 490 and 622 g-sec/cc which is a considerable increase over prior propellant compositions. Physical properties are changed; for instance, tensile strength is increased. Burning rate modifiers can be added to a basic composition in order to improve ballistic properties of the composition. The general purpose of this invention, therefore, is to produce a basic family of dense propellants which are extrudable or can be compression molded and which have suitable impulses that increased range results from their use in volume limited boost type application.

### SUMMARY OF THE INVENTION

The present invention is for an extrudable, high density solid propellant composition and its method of preparation. The composition consists essentially of a fluorocarbon binder, such as a copolymer of vinylidene fluoride and perfluoropropene (Viton) or a copolymer of vinylidene fluoride and trifluorochloroethylene (Kel-F elastomer), in the range of from 10 to 35 percent; elemental fuels and their hydrides or mixtures thereof, selected from the group consisting of aluminum, boron, zirconium, beryllium, titanium, magnesium, and their hydrides, in the range of from about 5 to 70 percent; and an oxidizer, generally an inorganic oxidizer selected from the group consisting of ammonium or alkali metal perchlorate in the range of from about 25 to 75 percent. The tradename designations given for the fluorine containing polymers useful herein are "Viton", a duPont de Nemours and Company polymer and "Kel-F Elastomer" available from the Minnesota Mining and Manufacturing Company. The composition is prepared by dissolving the fluorocarbon in a solvent such as acetone, then adding the oxidizer

and metal powder thereby forming a suspension. The suspension is then washed with a quantity of a precipitant for the fluorocarbon, in this instance hexane. The solid is permitted to settle and the liquid is decanted off. The solid is washed again with hexane after which the liquid is decanted off, the solid filtered and air dried or oven dried. The powder resulting is compression molded or extruded into the desired shape. The object of this method to produce an extrudable, high density solid propellant material which will have greater boost velocity than existing propellants. A product which is relatively safe to handle is formed and the process is amenable to large scale production of propellants, pyrotechnics, and explosive materials such as high energy, high density molding powders which can be molded or extruded.

Other objects and many attendant advantages of this invention will be readily appreciated as the same become better understood by reference to the following detailed description when considered in connection with the accompanying graphs.

### BRIEF DESCRIPTION OF THE DRAWINGS

- 25 FIG. 1 is a graph showing the theoretical impulse as a function of the basic composition;
- 30 FIG. 2 is a graph showing the theoretical impulse as a function of a zirconium modified basic composition;
- 35 FIG. 3 is another graph showing the theoretical impulse as a function of a beryllium modified composition;
- 40 FIG. 4 is yet another graph showing the theoretical impulse as a function of another modified basic composition; and
- 45 FIG. 5 is a graphic comparison of the boost velocities of fluorocarbon bound propellants with propellants containing conventional binders.

### DESCRIPTION OF THE INVENTION

In the present invention many compositions were studied, extruded, or pressed and fired. This invention is illustrated, but not limited, by the following basic composition consisting essentially of a fluorocarbon binder, such as a copolymer of vinylidene fluoride and perfluoropropene (Viton) and a copolymer of vinylidene fluoride and trifluorochloroethylene (Kel-F elastomer), in the range of from 10 to 35 percent; elemental fuels and their hydrides or mixtures thereof, such as aluminum, boron, zirconium, beryllium, titanium, magnesium, and their hydrides, in the range of from about 5 to 70 percent; and an oxidizer, generally an inorganic oxidizer such as ammonium or alkali metal perchlorate in the range of from about 25 to 75 percent.

In the use of very dense metals, less binder is required on a weight basis as the fuel volumes get smaller. For example, the density of boron is 2.34 g/cc, but the density of lead is 11.4 g/cc, and that of tungsten is 19.32 g/cc.

Oxidizers such as ammonium or alkali perchlorates and nitrates are interchangeable as far as processing is concerned. Calculations indicate that oxidizers such as hydrazine nitroformate will theoretically provide even better performance.

The following basic composition was modified as hereinafter described.

## Basic Composition

| Constituents         | Percent by weight |
|----------------------|-------------------|
| Ammonium perchlorate | 59                |
| Aluminum             | 21                |
| Viton A              | 20                |

The addition of various fuel mixtures to the above extrudable basic composition provided changes in burning rates which are shown in the following table. For example, the addition of copper, iron, boron, chromium, zirconium, or their derivatives at the 5 percent level in the basic composition showed significant burning rate changes:

TABLE I  
Burning Rate (in/sec.)

|                                                    | 1000 psi | 4000 psi |
|----------------------------------------------------|----------|----------|
| Basic formulation                                  | 0.47     |          |
| Extruded basic formulation modified by addition of |          |          |
| Ferrocene                                          | 0.70     | 1.5      |
| Copper                                             | 0.54     | 1.1      |
| Boron                                              | 0.72     | 1.65     |
| Chromium                                           | 0.5      | 1.1      |
| Copper Chromite                                    | 0.64     | 1.5      |
| Copper Stearate                                    | 0.56     | 1.2      |
| Copper Oxide                                       | 0.56     | 1.2      |
| Lead Salicylate                                    | 0.52     | 1.0      |
| Lead Resorcylate                                   |          | 1.10     |
| Titanium Dioxide                                   | 0.58     | 1.37     |
| Zirconium Boride                                   | 0.53     | 1.35     |
| Lead Carbonate                                     | 0.52     | 1.35     |

Mixtures of aluminum and zirconium as high energy, high density ingredients also produced significant changes in the burning rate of the extruded basic composition as shown in the following table:

TABLE II  
Burning Rate (in/sec.)

| Composition<br>(Percent by Weight) |    |      |    |      | Burning Rate<br>(psi) |        |      |
|------------------------------------|----|------|----|------|-----------------------|--------|------|
| Viton                              | AN | Al   | KP | Zr   | Tef                   | 1000AP | 4000 |
| 15                                 | 45 | 20   |    | 15   | 5                     | 0.60   | 1.35 |
| 15                                 | 45 | 20   |    | 20   |                       | 0.77   | 1.95 |
| 30                                 |    |      | 50 |      |                       | 0.47   | 1.22 |
| 20                                 | 80 |      |    |      |                       | 0.40   | 0.82 |
| 25                                 | 75 |      |    |      |                       | 0.40   | 0.84 |
| 15                                 | 85 |      |    |      |                       | 0.06   | 0.15 |
| 15                                 | 75 | 10   |    |      |                       | 0.45   | 0.92 |
| 16                                 | 50 | 20   |    | 10   | 4                     | 0.63   | 1.35 |
| 18.5                               | 45 | 16.5 |    | 16.5 | 3.5                   | 0.53   | 1.25 |

AP = ammonium perchlorate

AN = ammonium nitrate

Al = aluminum

KP = potassium perchlorate

Zr = zirconium

Tef = Teflon

Other modifications of the basic composition which showed significant changes in the burning are as follows:

## Modified Composition A

| Constituents         | Percent by weight |
|----------------------|-------------------|
| Viton                | 18.5              |
| Sodium azide         | 9.1               |
| Ammonium perchlorate | 54.6              |
| Aluminum             | 18.15             |

The sodium azide acts as a catalyst. Burn rate results of the extruded strands were as follows:

0.37 in/sec at 1000 psi

0.78 in/sec at 4000 psi

## Modified Composition B

| Constituents         | Percent by weight |
|----------------------|-------------------|
| Viton                | 25                |
| Magnesium            | 20                |
| Ammonium perchlorate | 55                |

Burn rate results of the extruded propellant were as follows:

0.54 in/sec at 1000 psi

1.07 in/sec at 4000 psi

The process by which the present invention is made uses a resin kettle with a fast propeller stirrer and a stiff rubber baffling device to prevent vortex formation. A stainless steel drum may be used to make larger batches. The required quantity of binder is placed in a container and dissolved in acetone or other suitable solvents such as methyl ethyl ketone and ethyl acetate. Approximately 25 cc of acetone per gram of Viton or Kel-F elastomer is used. Into this solution at room temperature are stirred the dry solid ingredients, the metal powder and oxidizer. After about 5 minutes of stirring the suspension a quantity of a precipitant for the fluorocarbon, about two and one-half times by volume of fluorocarbon solvent is added with stirring. Hexane was used in this instance. Other hydrocarbons such as petroleum ether may be used. After an additional 5 minutes of stirring, the solid is permitted to settle and the liquid is decanted off. Care must be taken at this point to prevent complete decantation, especially prior to the first washing. Residual solvent will permit easy agglomeration of the powder at this stage if most of the hydrocarbon evaporates off. The latter is detrimental to the preparation of a free-flowing molding powder which is suitable for extrusion. The remaining wet solid receives a second hexane wash after which it is decanted off, filtered and air dried or oven dried at 90° C. In this manner agglomeration is avoided. If a finer powder is desired, the second hexane wash may be decanted off and the wet solid screened. The powder after air drying and vacuum drying is compression molded or extruded into the desired shapes. The propellant surfaces not to be burned are inhibited prior to motor firing.

Referring now to the drawings, FIG. 1 is a graphic view of the theoretical specific impulse as a function of the basic formulation, as above set out, consisting essentially of Viton, aluminum, and ammonium perchlorate. FIG. 2 illustrates the theoretical specific impulse as a function of the composition wherein the basic formulation was modified by using zirconium as the elemental fuel in place of aluminum. In FIG. 3 the theoretical specific impulse as a function of the composition is shown in which beryllium was the elemental fuel used. FIG. 4 illustrates the theoretical impulse as a function of the composition wherein hydrazine nitroformate is the oxidizer with a fluorocarbon binder and the fuel, beryllium. FIG. 5 compares the boost velocities of fluorocarbon bound propellants with propellants bound with conventional binders such as polyurethanes and polyhydrocarbons. These conventional binders are designated by the symbol  $-\text{CH}_2-$ .

The performance of an ideal rocket, i.e., no pressure thrust, drag or gravitation or what may be termed "a gravitationless vacuum" is given by

$$V_{BO} = C_{av} \ln [m_t / (m_t - m_p)] ; \quad C_{av} = I_{sp} g$$

The logarithmic relation makes  $V_{BO}$  very dependent on a mass ratio. If the rocket were all propellant the  $V_{BO}$  would theoretically be infinite. Now if

$m_{BO}$  (mass of rocket at burnout) =  $m_t - m_p$   
and since,

$m_p$  = density of propellant,  $\rho_p \times$  volume of propellant,  
 $V_p$

$$m_t/(m_t - m_p) = (m_{BO} + m_p)/m_{BO}; 1 + m_p/m_{BO} = 1 + [\rho_p/(m_{BO}/V_{BH})]$$

so that

$$V_{BO} = I_{sp}g \ln (1 + [\rho_p/m_{BO}/V_p])$$

wherein

$V_{BO}$  = Velocity of rocket at propellant burnout

$C_{av}$  = Time average exhaust velocity (cm/sec) =  $I_{sp}$

$m_t$  = Total rocket mass at time zero

$m_p$  = Total propellant mass at time zero

$t$  = Time

$I_{sp}$  = Specific impulse

$g$  = Gravity

Since the mass of a rocket without propellant, and the volume to be occupied by the propellant generally are both fixed by design, the ratio  $m_{BO}/V_p$  (very often called the mass to volume ratio) is independent of propellant characteristics and actually characterizes the rocket or missile.

In FIG. 5 it is shown that the boost velocity ( $V_{BO}$ ) of fluorocarbon bound propellant is considerably better than the conventional binders.

The following table shows test results of several batches of propellants prepared in accordance with the present invention.

TABLE III

| Composition (percent by weight) |    |    |    | Composition by analysis, V/AP/Al/Zr | Measured density | Percent theoretical maximum density | Measured $I_{sp}$ |
|---------------------------------|----|----|----|-------------------------------------|------------------|-------------------------------------|-------------------|
| Viton                           | AP | Al | Zr |                                     |                  |                                     |                   |
| 20                              | 65 | 15 | —  | 22.08/63.39/14.53                   | 1.987            | 99.35                               | 238               |
| 20                              | 59 | 21 | —  | —                                   | 1.984            | 99.20                               | 228               |
| 20                              | 62 | 18 | —  | 21.98/60.48/17.54                   | 2.027            | 99.36                               | 239               |
| 20                              | 25 | —  | —  | 55.19/19.25/04.55/06                | 2.994            | 96.89                               | 149               |
| 20                              | 30 | —  | —  | 50.20/68/29.55/49.77                | 2.824            | 96.71                               | 162               |
| 20                              | 35 | —  | —  | 45.19.65/35.05/45.32                | 2.754            | 99.01                               | 175               |
| 20                              | 40 | —  | —  | 40.19.90/39.63/40.11                | 2.621            | 97.80                               | 194               |
| 20                              | 45 | —  | —  | 35.19.85/44.88/35.37                | 2.510            | 99.21                               | 196               |
| 20                              | 50 | —  | —  | 30.20.05/49.89/30.09                | 2.397            | 99.05                               | 200               |
| 25                              | 35 | —  | —  | 40.24.37/34.86/40.77                | 2.607            | 98.75                               | 185               |

AP = Ammonium perchlorate (100 $\mu$ ); V = Viton

Al = Aluminum

Zr = Zirconium

5 The invention described herein may be manufactured and used by or for the Government of the United States of America for governmental purposes without the payment of any royalties thereon or therefor.

What is claimed is:

10. The process for preparing an extrudable, high energy solid propellant comprising the steps of
  1. dissolving a copolymer of vinylidene fluoride and perfluoropropylene in acetone to form a solution;
  2. adding while stirring weighed quantities of a dry oxidizer selected from the group consisting of ammonium perchlorate, ammonium nitrate, potassium perchlorate and mixtures thereof and a fuel selected from the group consisting of aluminum, boron, beryllium, magnesium, and zirconium to form a homogeneous mixture;
  3. adding to said mixture while stirring a volume of hexane about three times the volume of said acetone;
  4. permitting said acetone and mixture to stand without stirring until all the solids settle;
  5. decanting off substantially all the liquid leaving a residue;
  6. washing the residue with hexane of about three times the volume of acetone;
  7. filtering out said residue;
  8. air drying the residue; and
  9. extruding said residue.

30 2. The process as defined in claim 1 wherein the oxidizer is ammonium perchlorate and the fuel is aluminum.

35 3. The process as defined in claim 1 wherein the oxidizer is ammonium perchlorate and the fuel is zirconium.

40 4. The process as defined in claim 1 wherein the oxidizer is ammonium perchlorate and the fuel is beryllium.

45 \* \* \* \* \*